

## UNITED STATES PATENT OFFICE

1,979,015

## STEEL ALLOY

Ernst Hermann Schulz, Dortmund, Germany, assignor to Vereinigte Stahlwerke Aktiengesellschaft, Dusseldorf, Germany

No Drawing. Application January 28, 1932, Serial No. 589,525. In Germany December 15, 1930

## 5 Claims. (Cl. 75—1)

This invention relates to a process for obviating or reducing cold shortness in steels containing phosphorus.

It is a known fact that as the phosphorus content in steels increases the tendency to cold shortness also increases, which is particularly evident in the scrap from the notched-bar toughness tests. Thus, according to Oberhoffer "Das technische Eisen" 1925, Springer, Berlin, phosphorus is classed as an undesirable element from the point of view of iron foundry work having regard to its undeniable action as a producer of cold shortness. Soft ingot steel is definitely brittle even when containing about 0.10% of phosphorus and when said steel contains more than 0.15% phosphorus, the measured value for the notched-bar toughness is so small as to render the steel useless for practical purposes.

It has unexpectedly been shown in accordance with the present invention that the addition of chromium (which otherwise exerts a hardening effect and therefore reduces rather than increases the toughness of the steel) will reduce to a great extent or entirely obviate the brittleness produced by the phosphorus.

Therefore the invention consists in a steel, containing between about 0.05 and 0.30% of carbon and a raised phosphorus content above 0.08% and for reducing the brittleness caused by the raised phosphorus content in addition thereto between about 0.25 and 1.5%, preferably 0.5 to 1% of chromium. The phosphorus content of the steel according to the invention lies preferably between about 0.08 and 0.17% and may be increased with increasing chromium content, so that with consequent increase of chromium content it may reach the highest amount of about 0.3% of phosphorus which is to be found in malleable iron.

The examples given hereinafter, relating to a steel containing about 0.10% of carbon clearly show the effects of the influence of chromium. The specific impact test (notched-bar toughness) is selected as a criterion for the toughness or brittleness together with the behavior of the test pieces under the impact test, such as is prescribed by the German State Railway Company for rail steels.

| 50<br>Phosphorus<br>percent | Chromium<br>percent | Notched-<br>bar tough-<br>ness m. kg.<br>per sq. mm. | Impact test                  |  |
|-----------------------------|---------------------|------------------------------------------------------|------------------------------|--|
|                             |                     |                                                      |                              |  |
| 55                          | 0.08                | 8                                                    | Not broken at the fifth blow |  |
|                             | 0.08                | 11                                                   | Not broken at the fifth blow |  |
|                             | 0.11                | 6                                                    | Broken at the fourth blow    |  |
|                             | 0.12                | 8                                                    | Not broken at the fifth blow |  |
|                             | 0.12                | 9.5                                                  | Not broken at the fifth blow |  |
|                             | 0.15                | 1                                                    | Broken at the first blow     |  |
| 60                          | 0.17                | 5                                                    | Not broken at the fifth blow |  |

It is readily apparent from these examples, that in the case of steels with phosphorus contents in which ordinarily the notched-bar toughness is reduced to quite negligible proportions and in which the rail impact test does not satisfy the 65 prescribed conditions, the notched-bar toughness can by the addition of chromium be increased to a value which is a multiple of that of the steel without chromium and the impact test can be made to satisfy the prescribed requirements by 70 the addition of chromium to said steel.

It is possible to bring out this effect produced by the chromium content to a more pronounced degree the lower the carbon of the steel and the lower the inherent brittleness thereof, the 75 process being primarily applicable to steels containing up to about 0.3% of carbon. In this connection it is an advantage to increase the chromium content as the phosphorus content increases.

I claim:—

1. A steel alloy containing between about 0.05 and 0.3% of carbon and between about 0.5 and 0.75% of chromium for reducing the brittleness caused by a phosphorus content between about 85 0.08 and 0.17%, the balance of the alloy consisting substantially of iron.

2. A steel alloy containing between about 0.05 and 0.3% of carbon and between about 0.25 and 1.5% of chromium for reducing the brittleness 90 caused by a phosphorus content between about 0.08 and 0.17%, the balance of the alloy consisting substantially of iron.

3. A steel alloy containing between about 0.05 and 0.3% of carbon and between about 0.5 and 0.75% of chromium for reducing the brittleness 95 caused by a phosphorus content between about 0.08 and 0.3%, the balance of the alloy consisting substantially of iron.

4. A steel alloy containing between about 0.05 and 0.3% of carbon and between about 0.25 and 1.5% of chromium for reducing the brittleness caused by a phosphorus content between about 100 0.08 and 0.3%, the balance of the alloy consisting substantially of iron.

5. A steel alloy containing between about 0.05 and 0.3% of carbon and between about 0.5 and 0.75% of chromium for reducing the brittleness 110 caused by a phosphorus content between about 0.08 and 0.17%, the balance of the alloy consisting substantially of iron, the chromium content being increased as the phosphorus content increases.

ERNST HERMANN SCHULZ.

115

120